

Feb. 16, 1926.

**1,573,499**

J. M. NICOL

## CENTRIFUGAL SEPARATION

Filed Sept. 26, 1923



Fig. 2.



John Malcolm Neaf Inventor  
By his Attorneys  
Brundage, Wright, Neaf & Bear

## UNITED STATES PATENT OFFICE.

JOHN M. NICOL, OF MILL VALLEY, CALIFORNIA.

## CENTRIFUGAL SEPARATION.

Application filed September 26, 1923. Serial No. 665,007.

*To all whom it may concern:*

Be it known that I, JOHN MALCOLM NICOL, a subject of the King of Great Britain, a resident of Mill Valley, in the county of 5 Marin and State of California, have invented a certain new and useful Centrifugal Separation, of which the following is a specification.

This invention relates to a process of centrifugal separation and more particularly to a process of centrifugally separating mixed materials, ores, minerals, or fine ore slimes.

The invention has as an object the separation of ores or minerals from each other such as are difficult or expensive to separate by flotation processes or other means. It has also as an object the separation of mixed slime sulphide concentrates from oil flotation processes where selective flotation has failed of application or where the slimes are too fine to treat by wet table concentration. A further object is to make a substantially quantitative separation of such 20 ores or minerals and to accomplish this rapidly and relatively inexpensively. Furthermore, a special object of the invention is to separate noble metals like gold and platinum from associated minerals by a centrifugal process. Further objects of the invention 25 will become apparent as the description proceeds.

In accomplishing these objects and carrying out the invention I employ centrifugal force to act upon the materials and to arrange them in concentric layers of progressively varying densities. In order to obtain the most efficient centrifugal action it is desirable to treat the materials in a finely 30 comminuted or divided state, preferably in the form of fine aqueous pulp or in the form of slimes. Although the separation of the different minerals into concentric layers by centrifugal force is both effective and rapid, the difficulty in the practical application of 35 this method to the art has consisted in obtaining a substantially complete separation of the different layers from each other, and especially in obtaining a continuous discharge of the individual concentrates as 40 separate products. As far as the difficulty has resided in a proper form of apparatus, I believe I have solved this phase of the matter by the invention disclosed in my application, Serial No. 659,727 of August 28, 1923,

wherein I have disclosed a centrifugal machine of well-balanced construction having an inner fixed or rotatable bowl for causing a differential movement of the materials, and having an upper adjustable bowl for providing two cutouts for the mineral layers. Apparatus is designed also to operate with a column or wall of mercury subjected to rapid rotation for the purpose not only of allowing the aqueous mixture or pulp to 60 pass freely upwardly, but also of collecting heavy metals like gold.

By way of a more detailed description of the apparatus reference is made to the accompanying drawing, in which,

Fig. 1 represents a vertical central section of the centrifugal separator; and

Fig. 2 represents a modification of a part of the structure comprising the inner bowl.

In the drawings there is shown a main 75 supporting frame 1 that carries an upper cross member 2 and a lower cross member 3. The upper cross member carries a removable angle bracket 4 serving as the supporting means for an upper bearing, and the lower 80 cross member carries another removable angle bracket 5 serving to support a lower bearing, these bearings serving to support the revolving parts to be described later. There is also provided a footstep block 6 85 having an oil well 7 and an adjustable center pivot 8, and a preferably brass bushed central vertical bearing 9.

The main revolving member in which the 90 centrifugal effect is produced consists of a bowl 10 into the bottom of which is screwed a footstep shaft 11 held by a set screw 12. The shaft 11 revolves freely in the bearing 9 and rests on the pivot of the screw 8, this mechanism being finely balanced so that the 95 bowl will not revolve irregularly during operation. The said bowl is provided with two interior annular ruffles 13 and 14 and a large annular concave ruffle 15 designed to contain mercury in this particular embodiment. There is also a discharge orifice 16 provided with a removable plug.

A central vertical feed pipe 17 is screwed into the bottom of the bowl 10 at a socket 18, and is provided with three openings near the said socket, one of which, 19, is shown. Said pipe 17 also serves as the driving member for the bowl 10, and for this purpose is provided with a driving pulley 20. The upper end of the pipe 17 revolves in a bear- 105

ing 21 which is fitted into and held in place by a non-rotating vertical pipe 22. The latter fits into a center hole in the bracket 4, and is supported by a removable threaded 5 collar 23. The lower end of the pipe 22 is threaded into a socket in a stationary massive ring 24, which is maintained in concentric relationship with the central revolving pipe 17 of the bowl 10 by means of a 10 center bushing 25 serving as an inner bearing. On the outside of the fixed pipe 22 is located a simple clamp collar 26, held with set screws, and a flat disc 27 is located thereon and connected to the massive ring 24 by 15 a short cylindrical section of pipe 28. The three members 24, 27 and 28, are joined together and supported by the pipe 22, as will be evident, thus forming a single non-rotating member, which may be termed an 20 inner guide bowl. As will be seen, this is stationary in the embodiment now being described.

Above the disc 27 is provided a ball bearing 29 on which runs an upper rotating hood bowl 30, which is suitably connected to and driven by a horizontal pulley 31 provided with a bearing 32. Said hood bowl 30 has an inner annular concave groove 33 that is provided with a number of discharge openings such as 34.

It will be seen that the space between the lower bowl 10 and the upper hood bowl 30 represented by numeral 35 constitutes an annular discharge orifice for the concentrates of higher density congregating against the inside of the bowl 10, and this space 35 may be decreased or increased by manipulation of the screw 8 so that an opening as fine as  $1/100''$  may be obtained.

40 A noteworthy feature of this structure is that such a fine adjustment may be made during the operation of the apparatus, thereby making it possible to obtain a clean separation during the running of the machine by observation of the nature and quality of the concentrate issuing through said opening 35. The discharge of concentrates coming through the annular opening 35 will fall into a suitably placed launder shown at 36. The concentrates lying inside of the outer ring of heavier concentrates may be made to pass out through the openings 34 and will be discharged into an outer launder shown at 37.

55 A wooden plug 38 may be inserted in the bottom of the pipe 17 to close the same below the orifices 19.

In Fig. 2 a modification is illustrated, showing a construction in which the inner bowl may be made rotatable. A cross member 2' carrying a bracket 4' supports a bearing 21' around a centrally fitted pipe 17'. A central pipe 22' is mounted over the said bearing 21' and has screwed at the upper end thereof a driving member 39 rotat-

ing upon ball bearing 40. A bearing 41 inserted in the bracket 4' serves to guide pipe 22'. The latter is therefore made rotatable and consequently the corresponding massive ring and inner bowl, described in detail in the above embodiment, will be made rotatable, all other parts of the structure being the same as in the above-described preferred embodiment. 70

In centrifugal methods the principal difficulty has been to separate the different layers owing to the thinness of some of them, since it is almost mechanically impossible to effect a cutout of such a thin layer, and it is furthermore impossible to effect a mechanical cutout of thick layers since there will be intermingling of materials. For example, in the case of silver-lead, pyritic and zinc ore, the particles of the silver-lead slimes would have a specific gravity of about 7 and would form the outer layer and probably would not exceed 1/100 of an inch in thickness. The next layer would be the pyritic material having a specific gravity of 4.5, which layer would be generally thicker. To separate these two layers by mechanical means is obviously hopeless.

In order to effect a substantially complete separation of such layers resulting from a centrifugal process, I have invented a means of so conducting the process that the region within which a cutout may be made is substantially widened so that a very thin layer may be completely removed from the adjacent layer. Accordingly the fundamental idea of the invention consists in adding another material or mineral to the mixture to be treated in the centrifuge, which material may be either a natural product or an artificial one having a density between the respective densities of the two minerals to be separated; the object of this addition is to increase the bulk of material between the layers so that a wide zone will exist between the minerals and a clean cutout can easily be made.

The invention may obviously be carried out in a multitude of ways widely dissimilar as to minerals and separating media and, therefore, it will suffice to give a few examples with respect to particular ores and minerals. For example, in the case of the silver-lead, pyritic, zinc ore mentioned, barytes may be added to the mixture to form a dividing medium between the silver-lead and the pyritic minerals, inasmuch as it has a density of about 5. The order of the concentric columns of ascending pulp would then be: 1. silver lead, 2. barytes, 3. pyritic materials, and 4. the remainder of the inner concentric columns. By using the apparatus above referred to two groups of products would be obtained, namely, first, the silver-lead concentrate with part of the barytes, and second, the remainder of the 115 120 125 130

barytes, together with the rest of the material in the form of a mixed product. By taking the first product and passing it through a simple flotation cell the barytes 5 would be thrown down and could be used over again in a closed metallurgical circuit and the silver-lead product would then be delivered as a clean concentrate.

The dividing media should preferably be 10 neutral with regard to subsequent metallurgical treatments. For example, the barytes suggested above as a medium is not affected by flotation, whereas silver-lead concentrates are readily amenable to flotation. 15 Magnetite is another suitable medium inasmuch as it can be used between non-magnetic sulphides and can subsequently be separated out by magnets and then returned for re-use. If the medium used can be obtained in 20 abundance and cheaply it might be possible in many cases to omit the separation of the medium and concentrate and to smelt them together directly. In order to obtain a suitable density it may be desirable to manufacture 25 a suitable medium by grinding together suitable minerals having the proper densities or by providing any other suitable material having the required density. The question of the selection of media depends 30 entirely upon the nature of the minerals or ores being treated and the character of subsequent operations.

As a still further example of a mineral treatment may be given an ore carrying the 35 following materials: gold, free and in fracture planes of pyrites and arsenical pyrites; complex silver sulphides and arsenides together with tellurides of silver and gold; galena, associated with gold and silver sulphides; antimonial silver, occurring as 40 stephenite or tetrahedrite; zinc, sulphide or sphalerite; molybdenite; pyritic minerals. In this particular art the minerals of economic importance are gold, molybdenum, 45 silver-lead, and possibly zinc. By the use of the centrifugal machine gold would be driven into the mercury layer with or without amalgamation, amalgamation not being essential in this process; the silver sulphides 50 and arseno-minerals with the exception of tetrahedrite, would pass with the galena and may be separated out by a dividing medium consisting of ilmenite having a density of 5. The first treatment would, therefore, result in: 1. gold; 2. silver-lead concentrate carrying some arsenical pyrites, together with a portion of the ilmenite; 3. the 55 remaining ilmenite, plus a mixed pyritic concentrate and tailings carrying also the sphalerite and molybdenite. Product No. 2 could be directly treated or sold as it is of value, while product No. 3 would be passed through a second centrifugal machine, using this time as a dividing medium either celestite 60 or a selected garnet sand or a hematite

sand or an artificial product having a density of 4 to 4.2. There would then result from this third product two sub-products as follows: (a) a pyritic concentrate carrying tetrahedrite and the molybdenite, (b) sphalerite and any middlings or tailings 70 sands. This is as far as it would be advisable to go with the centrifugal separation, since the pyritic group and the molybdenite are too near in their respective densities. 75

It will be apparent in considering the above example that an ore or mineral mixture may be advantageously and successfully treated by the above described centrifugal process, whereas it would be economically impossible to do much with such an ore by means of any other known process. Many other adaptations of the invention will suggest themselves to those skilled in the art 85 upon considering the use of the above process, particularly in connection with my centrifugal machine above mentioned.

As many apparently widely different embodiments of my invention may be made 90 without departing from the spirit thereof, it is to be understood that I do not intend to limit myself to the embodiments described except as defined in the following claims.

I claim:—

1. The process of substantially completely separating mineral particles having different densities, comprising adding thereto a material having an intermediate density and centrifugalizing the mix to obtain concentric layers with the added material positioned between the minerals to be separated, and effecting a cutout of a mineral layer at some point within said intermediate layer between the planes of the outer layers. 100

2. The process of claim 1 wherein the centrifugalizing is performed within a substantially vertical rotating column of mercury at the top of which is provided a cutout for the outer mineral layer. 105

3. The process of claim 1 wherein the minerals are given a differential movement during centrifugalizing. 110

4. The process of claim 1 wherein the minerals are in the form of a fine ore pulp containing considerable quantities of mixed sulphide concentrates. 115

5. The process of claim 1 wherein the minerals are in the form of a fine ore pulp containing sulphides of silver-lead and zinc, 120 and pyrites, and the first cutout is a silver-lead concentrate.

6. The process of separating mineral particles consisting in adding to a mixture of such particles a material of specific gravity 125 intermediate the specific gravity of such particles and non-responsive to selective flotation, stratifying the mixture according to specific gravity, cutting out a layer from the stratified mass and subjecting the mate- 130

4  
rial so cut out to selective flotation to separate the desired mineral from non-flotative and added matter.

5 7. The process of separating mineral particles having different densities, comprising subjecting them to centrifugal action in the form of an aqueous finely sub-divided mixture in contact with an outer rapidly rotating wall of mercury along which the materials pass, and are formed into layers, and thereupon effecting a cutout in said layers at the top of the wall of mercury between the planes of the outer layers.

10 8. The process of substantially completely separating mineral particles having different densities comprising adding thereto a non-mercurial material having an intermediate density and centrifugalizing the mix in contact with a rotating wall of mercury to obtain concentric layers with the added material positioned between the minerals to be separated, and effecting a cutout of a mineral layer at some point within said intermediate layer.

15 9. The invention in claim 8 wherein the cutout is above the top of the wall of mercury.

20 10. The process of substantially completely separating mineral particles having different densities comprising adding thereto a non-mercurial material having an intermediate density and progressively introduc-

ing and centrifugalizing the mix in relatively thin layers in contact with a rotating wall of mercury to obtain concentric 35 layers with the added material positioned between the minerals to be separated, and effecting a cutout of a mineral layer at some point within said intermediate layer.

40 11. The process of separating mineral particles having different densities, comprising adding thereto a material having an intermediate density and centrifugalizing the mix to obtain relatively thin concentric layers with the added material positioned 45 between the minerals to be separated, and effecting a cutout of a mineral layer at the top of the layer and at some point within said intermediate layer between the planes of the outer layers.

50 12. The process of separating mineral particles having different densities, comprising subjecting them in the form of a finely divided mixture containing added non-mercurial material, to centrifugal action in contact with a rotating wall of mercury, causing the minerals to form into thin concentric layers inside of the mercury wall, and effecting a cutout in a layer between the planes of the outer layers.

55 In testimony that I claim the foregoing, I have hereunto set my hand this 24th day of September, 1923.

60 JOHN M. NICOL.